

March 30, 1937.

R. R. SMITH

2,075,066

METHOD OF ROLLING METAL

Filed Sept. 15, 1934



INVENTOR.

RUSSELL R. SMITH.

BY

*Alvin A. Brown*  
ATTORNEYS.

## UNITED STATES PATENT OFFICE

2,075,066

## METHOD OF ROLLING METAL

Russell R. Smith, Ashland, Ky., assignor to The  
American Rolling Mill Company, Middletown,  
Ohio, a corporation of Ohio

Application September 15, 1934, Serial No. 744,245

8 Claims. (Cl. 29—19)

My invention has to do with the rolling of rough plate or thin bar to useful finished gauges, and has for its principal object the provision of a new and improved method of reduction for 5 such material, permitting the securing of lighter gauges with less tendency to pinching. The ancillary objects of my invention will be pointed out hereinafter or will be apparent to one skilled in the art upon reading these specifications, 10 wherein I have described my novel process in an exemplary embodiment. In the drawing I have shown the several steps of my process in a dia-grammatic way.

The terms "rough plate", "thin bar" and the 15 like have been applied to the material produced from slabs on the modern continuous hot mill, or to equivalent material otherwise produced. Such material can be produced at a cost per 20 pound substantially the same as that of sheet bars produced on the blooming mill; but it is of much thinner gauge. It has therefore been seen that this material would form advantageous starting pieces for non-continuous reduction steps producing thin gauges. The product of the 25 continuous hot mill can be had in different gauges. The gauges mentioned hereinafter are exemplary but not limiting; and I shall refer to the hot mill product for convenience as thin bar in these specifications, not intending thereby to imply any gauge limitation. The thin bar may be produced, of course, either on a hot strip mill, a continuous tandem mill or a single stand mill.

Certain problems arise in connection with the 30 use of this material. Inasmuch as the width that can be produced on the hot mills is limited, the practice is to shear the thin bar into pieces the length of which is representative of the width of the desired finished sheet, and then 35 cross roll the pieces. For example, it is desired to produce a sheet 66 inches wide by 100 inches long and .037 inch thick. The thin bar for such a sheet might be rolled to .081 inch in thickness and 53 inches wide. The stock 40 would then be sheared 68 inches long. But in cross rolling thin bar as thin as .081 inch (which in packs of two is only .162 inch thick) it is very difficult to prevent pinching, especially because the pack has no convexity in the direction of the 45 mill rolls during cross rolling, and is of uniform gauge or thickness across the entire 68 inches of its width. In the language of the roller, "the pack has no middle."

A practical way of overcoming this difficulty, 50 has been practiced in the art; but involves the use of thicker thin bar. The thin bar has been rolled to a thickness of .109 inch, and to a correspondingly narrower width, such as 36 inches. The bar was then sheared to a length of 67 55 inches. Such material matched for a pack of

two gives a pack thickness of .218 inch at the outset. This pack is thick enough so that the roller, in cross rolling it, can take a heavy draft on the first pass. The rolls are then deflected sufficiently to give the pack a middle, by making 5 it .004 to .005 inch thicker in the center than at its edges. This permits finishing to the lighter gauge with much less danger of pinching. But, starting with such thin bar, the thickness of the 10 pack requires 7 to 9 passes to reduce it to a 16 gauge breakdown and 7 to 9 passes more to reduce the breakdown to a 20 gauge sheet.

My novel process solves these problems as I shall hereinafter describe. I start preferably, though not necessarily, with a wide thin bar, 15 stock which will be relatively thick, because I do not shear it into pieces as long as the desired width of the finished sheet. I either employ thin bar which already has a convexity due to continuous hot rolling methods, or I give it a convexity or middle by an after treatment. This may conveniently be done by giving it a hot rolling pass with the center of the thin bar artificially cooled by water or other means. It may 20 of course be done in other ways known to the 25 art.

I then shear the thin bar into pieces shorter than the desired width of the finished sheet. The sheared pieces are then cross rolled to bring them to a length at least equal to the width of the 30 desired finished sheet. During this first cross rolling there will be no convexity longitudinally of the mill; but the convexity longitudinally of the piece will not be destroyed. Due to the comparative shortness of the sheared pieces, this first cross 35 rolling may be carried on in a narrow mill, thus relieving the wide mill of duty, and permitting the continued use of narrow mill equipment already purchased. Usually one or two passes are 40 all that are required to elongate the thin bar to the desired length. If these passes are taken immediately after the formation and shearing of the thin bar, they may usually be taken as a part 45 of the thin bar formation process, and without reheating. The thin bar pieces may usually be matched after the shearing and rolled in pairs in the first cross rolling.

The thin bars or packs are reheated for the final 50 reduction steps, which comprise a second cross rolling. That is to say, the packs are again turned through an angle of 90 degrees. This gives a pack or piece adapted for rolling on a wide mill in the direction of the pack's shorter dimension, the longer dimension of the pack being as long as 55 the width of the desired finished sheet. The longer dimension of the pack is the direction of width of the original thin bar pieces. Consequently my pack differs from packs previously produced in that it initially has convexity longitudinally of the wide mill. It does not require a 60

special convexity producing treatment, nor does it have to be so thick as to permit of such treatment. The second cross rolling is continued until the pack is down to finished gauge.

5 In the drawing, 1 represents a hot mill, or the end element of a hot mill train, producing thin bar. Or it may be a special mill, or representative of a special pass to form convexity in thin bar. A piece of sheared thin bar is shown at A. It has 10 convexity, the edges being thinner than the middle. The piece A, or a matched pair of the pieces A are turned through an angle of 90 degrees into the position B and cross-rolled through a mill 2 (which may be a narrow mill) to form the elongated piece or pack C. This pack or piece has 15 convexity in the direction in which it was cross rolled, but none longitudinally of the rolls of the mill 2. It will be of a length at least equal to the width of the desired finished sheet. The piece 20 or pack C is next rolled through a mill 3 in a direction which is cross, or at right angles to, the direction of the first cross rolling, to form the finished product D.

In carrying out my process, by way of example, 25 in producing an order of sheets 66" wide by 100 inches long, and .037 inch thick, the piece A would be 54 inches wide and sheared to a length of 54 inches. It would average .104 inch thick, but would be, say, .107 inch thick in the center and 30 but .102 inch thick at the edges. A pair of the thin bars A would be matched and turned as at B, giving a pack averaging .208 inch thick with convexity in the direction of roll length during cross rolling. When rolled in the mill 2 it 35 would be elongated say from 54 inches to 71 inches, the thickness of the ends of the pack being reduced from .102 to .077 inch, while the thickness of the mid-portion would be reduced from .107 to .081 for each piece in the pack. Upon the 40 positioning of the pack for the second cross rolling these ends become the edges of the pack, which will be .154 inch thick while the center of the pack will be .162 inch thick, giving plenty of convexity.

45 The pack C is carried down to gauge in mill 3 in 5 to 7 passes, which elongate it to 106 inches. The convexity of the pack permits reduction to light gauges without pinching.

Modifications may be made in my invention 50 without departing from the spirit thereof.

Having thus described my invention, what I claim as new and desire to secure by Letters Patent, is:—

1. A method of producing thin bar packs or 55 pieces for reduction to sheet gauges and with initial convexity which comprises starting with thin bar stock having convexity but less in width than the desired width of finished sheets, shearing the thin bar stock into thin bars, elongating 60 the thin bars transversely until the length thereof equals the desired width of the finished sheets without destroying the original convexity, and afterward elongating them in the original direction of rolling.

65 2. A method of producing sheet metal from thin bar which comprises providing wide thin bar stock with initial transverse convexity, shearing the stock into pieces shorter than the desired width of finished sheets, rolling the pieces in a direction 70 transverse to the direction of rolling of the original thin bar stock to bring them to a gauge suit-

able for single part reduction and a length at least equal to the desired width of finished sheets but without destroying the original convexity, and finally rolling the material to gauge in a direction parallel to the direction of rolling of the thin bar stock. 5

3. A method of producing sheet metal from thin bar which comprises providing thin bar stock with initial transverse convexity, shearing the stock into thin bars, matching the thin bars into packs 10 and rolling them in a direction transverse to the direction of rolling of the thin bar stock to increase the width of the material (as respects the direction of original rolling) to the width of the desired finished sheets but without destroying the original convexity, and afterward rolling the widened material down to gauge in the direction 15 of original rolling of the thin bar stock.

4. A method of producing sheet metal from thin bar, which comprises providing thin bar stock 20 with initial transverse convexity, shearing the stock into pieces shorter than the desired width of finished sheets, rolling the pieces in a direction transverse to the direction of rolling of the thin bar stock to bring them to a length at least equal 25 to the desired width of finished sheets, whereby starting pieces are formed for a second rolling in a direction parallel to the direction of rolling of the thin bar stock, said pieces having convexity in the direction of their length, and finally rolling 30 said pieces to gauge in a direction parallel to the direction of rolling of the thin bar stock.

5. A method of producing sheet metal from thin bar, which comprises providing thin bar stock 35 with initial transverse convexity, shearing the stock into thin bars, matching the thin bars into packs and rolling them in a direction transverse to the direction of rolling of the thin bar stock to increase the width of the material (as respects the direction of original rolling) to the 40 width of the desired finished sheets, re-heating the elongated packs and rolling them down to gauge by a second rolling operation in a direction parallel to the direction of rolling of the thin bar stock. 45

6. The method of claim 5, wherein the first mentioned transverse rolling is carried on in a narrow mill, and the second mentioned rolling is carried on in a wide mill.

7. A method of preparing wide, convex pieces 50 from narrow, transversely convex, thin bar stock, which comprises cutting thin bar stock which is narrower than the desired width of finished sheets into pieces, rolling these pieces in a direction transverse to the direction of rolling of the thin bar stock, so as to widen them to at least the desired width of finished sheets while preserving 55 their initial convexity in the initial direction, whereby pieces are provided which, if rolled in a direction parallel to the direction of original rolling of the thin bar stock, will have a dimension transverse to the direction of said final rolling, which is at least equal to the width of the desired 60 finished sheets, and which will have a substantial convexity in the proper direction for such rolling. 65

8. The method of claim 7, wherein the said transverse rolling of the thin bar pieces is carried on immediately after the formation of the thin bar material by hot rolling, and as a part of the same heat.

RUSSELL R. SMITH.